

## UNITED STATES PATENT OFFICE.

PAUL D. MERICA, OF NEW YORK, N. Y., ASSIGNOR TO THE INTERNATIONAL NICKEL COMPANY, OF NEW YORK, N. Y., A CORPORATION OF NEW JERSEY.

## NICKEL ALLOY AND METHOD OF MAKING THE SAME.

No Drawing.

Application filed June 26, 1923. Serial No. 647,911.

To all whom it may concern:

Be it known that I, PAUL D. MERICA, a citizen of the United States, residing in New York, in the county of New York and

5 State of New York, have invented a new and useful Improvement in Nickel Alloys and Methods of Making the Same, of which the following is a full, clear, and exact description.

10 This invention relates to nickel alloys and method of making the same, and particularly to alloys of aluminum and nickel or of aluminum and Monel metal, which is a trade name for a natural nickel and copper 15 alloy made by The International Nickel Company.

I have found that the addition of aluminum to nickel or nickel-bearing metals, such as Monel metal, has a great effect on the 20 physical properties thereof. The resulting alloy has a high tensile strength and is highly resistant to erosion and corrosion. It is therefore particularly valuable for use in steam turbine blading or in other applications 25 where these properties are desirable.

In the manufacture of this alloy, I take molten nickel or Monel metal and deoxidize it, preferably with magnesium. The deoxidized metal is then mixed with molten 30 aluminum in the proper proportions. To facilitate a thorough mixing, I pour the principal melt, that is, the nickel or nickel-bearing metal, onto the aluminum. This pouring of the heavier metal onto the lighter 35 insures thorough mixing and uniform composition.

The mixing of the metals produces a marked evolution of heat which raises the temperature of the ladle considerably. I 40 utilize this extra heat by allowing the molten alloy to stand for a period of three to five minutes, thus giving the impurities an opportunity to rise to the surface and separate from the metal. The amount of heat 45 evolved is roughly proportional to the percentage of aluminum added.

The clean metal is then poured into ingots which are reduced to shapes by the processes usual in nickel and Monel metal practice. 50 The surface of the ingots must be removed prior to rolling, and with an aluminum content of under 3% or 4% the surface may be chipped or planed off. When the aluminum content is higher, it is necessary to 55 grind the ingots.

After heating and rolling, aluminum Monel alloys containing as much as 5% aluminum can be machined with ordinary tools.

The addition of aluminum increases both 60 the hardness and tensile strength of the metal. The best mechanical properties are obtained with aluminum between 3% and 5%, although amounts above 1% are effective. The upper limit of the aluminum content depends largely on the properties desired. Good results may be had up to 10%, although there is great difficulty in grinding and reducing ingots containing so much 65 aluminum. If the aluminum content is increased above 17%, the alloy is very brittle.

With an aluminum content between 3% and 5%, hot rolled rods may be produced with a true proportional limit of as high as 80,000 pounds per square inch, which would 70 be reduced by dead annealing at 1650° F. to not less than 60,000 pounds per square inch. High temperature tests show that the alloy retains its strength very satisfactorily at 750° F., and in fact the percentage reduction in the proportional limit at this temperature as compared with ordinary temperatures is less than in the case of Monel 75 metal. The resistance to corrosion is as great as, or greater than, in Monel metal.

The addition of carbon to the alloy between 0.1% and 0.5% exercises a marked effect in increasing the hardness and tensile strength.

While I prefer to use Monel metal, which 90 is the natural alloy consisting of 68% to 70% nickel, a small percentage of iron and the remainder copper, I may use nickel and copper in other proportions, as, for example, 50% to 80% nickel and 20% to 40% copper, 95 together with aluminum in the desired amount. The addition of .25% to 2.5% manganese is also desirable. The alloy apparently is not greatly affected by the presence of other metals in small amounts as 100 may occur on account of impurities in the metals used.

While I have described the preferred embodiment of my invention, it will be understood that it is not limited thereto but may 105 be otherwise embodied within the scope of the following claims.

I claim:

1. The method of making nickel alloys, which includes deoxidizing the principal 110

- melt and then mixing it with molten aluminum.
2. The method of making nickel alloys, which includes deoxidizing the principal melt with magnesium and then mixing it with molten aluminum.
3. The method of making nickel alloys, which includes mixing the principal melt with aluminum and utilizing the evolved heat to maintain the alloy at or above a pouring temperature over a settling period, thereby giving impurities in the alloy time to separate therefrom.
4. The method of making nickel alloys, which includes deoxidizing the principal melt, mixing the principal melt with aluminum, and utilizing the evolved heat to maintain the alloy at or above a pouring temperature over a settling period, thereby giving impurities in the alloy time to separate therefrom.
5. The method of making nickel aluminum alloys, which includes pouring the nickel melt onto the aluminum.
6. An alloy containing the elements which go to make up Monel metal and aluminum, containing from 1% to 10% of aluminum.
7. An alloy containing the elements which go to make up Monel metal and aluminum, containing from 1% to 10% of aluminum and containing carbon from .1% to .5%.
8. An alloy containing 50-80% nickel, 20-40% copper, 1-10% aluminum, and 0.25-2.5% manganese.
9. An alloy containing 50-80% nickel, 20-40% copper, 1-10% aluminum, 0.25-2.5% manganese, and 0.1-0.5% carbon.
10. An alloy of nickel, copper and aluminum, wherein the content of nickel is in excess of 50% and the content of aluminum is not less than about 3% and not more than 17%, the predominant metal of the remaining content being copper.
11. An alloy of nickel, copper and aluminum, wherein the content of nickel is not less than 55%, the content of copper is not less than 18%, and the content of aluminum is not less than about 3%, the three metals named forming the predominant percentages of the alloy.
12. An alloy of nickel, copper and aluminum, wherein the content of nickel is not substantially less than 50% and the content of aluminum is about 4% to 5%, the predominant metal of the remaining content being copper.
13. An alloy of nickel, copper and aluminum, wherein the content of nickel is 60% to 70% and the content of aluminum is 10% to 3%, the predominant metal of the remaining content being copper.
14. An alloy of nickel, copper and aluminum, wherein the content of nickel is in excess of 50% and the content of aluminum is not less than about 3% but is insufficient to destroy the malleability of the alloy for mechanical working, the predominant metal of the remaining content being copper.
15. An alloy of nickel, copper and aluminum, wherein the content of nickel is not less than 50% and the content of aluminum is between 1% and 17%, the remaining content consisting essentially of copper.
16. An alloy containing 1%-17% of aluminum, the remainder consisting essentially of nickel and copper with the nickel in excess of the copper, the copper being not less than 18%.
17. An alloy consisting essentially of 50%-80% nickel, 20%-40% copper, and 1%-10% aluminum.
18. An alloy consisting essentially of 50%-80% nickel, 20%-40% copper, and 1%-10% aluminum, together with carbon not in excess of .5%.
19. An alloy containing the elements which go to make up Monel metal and aluminum containing from 1% to 10% of aluminum, together with carbon not in excess of .5%.
- In testimony whereof I have hereunto set my hand.

PAUL D. MERICA.